

A. E. SPINASSE,  
METHOD OF AND APPARATUS FOR DRAWING GLASS,  
APPLICATION FILED OCT. 16, 1915.

1,336,056.

Patented Apr. 6, 1920.

5 SHEETS—SHEET 1.



(Witness)

३३५

Chas. L. Stauffer

Attorney

1,336,056.

A. E. SPINASSE.

METHOD OF AND APPARATUS FOR DRAWING GLASS.

APPLICATION FILED OCT. 16, 1915.

Patented Apr. 6, 1920.

5 SHEETS—SHEET 2.

Fig. 5.



Fig. 7.



By



Fig. 9.



Char. L. Stauffen

Attorney

A. E. SPINASSE.

METHOD OF AND APPARATUS FOR DRAWING GLASS.  
APPLICATION FILED OCT. 16, 1915.

1,336,056.

Patented Apr. 6, 1920.

5 SHEETS—SHEET 3.

FIG. 6.



FIG. 10.



58 A

FIG. 11.



FIG. 12.



Inventor

—Arthur E. Spinasse—

Witness

By

Charles L. Stauffer

Attorney

A. E. SPINASSE.

METHOD OF AND APPARATUS FOR DRAWING GLASS.  
APPLICATION FILED OCT. 16, 1915.

1,336,056.

Patented Apr. 6, 1920.

5 SHEETS—SHEET 4.

FIG. 13.



FIG. 14.



FIG. 15.



Inventor

—Arthur E. Spinasse—

Witness



By



Attorney

A. E. SPINASSE.

METHOD OF AND APPARATUS FOR DRAWING GLASS.  
APPLICATION FILED OCT. 16, 1915.

1,336,056.

Patented Apr. 6, 1920.

5 SHEETS—SHEET 5.

FIG. 16.



FIG. 17.



FIG. 18.



FIG. 19.



FIG. 20.



FIG. 21.



FIG. 22.



FIG. 23.



FIG. 24.



FIG. 25.



FIG. 27.



Inventor

Arthur E. Spinasse —

Witness



By

  
Lehar. C. Stauffer  
Attorney

# UNITED STATES PATENT OFFICE.

ARTHUR E. SPINASSE, OF MOUNT VERNON, OHIO.

## METHOD OF AND APPARATUS FOR DRAWING GLASS.

1,336,056.

Specification of Letters Patent.

Patented Apr. 6, 1920.

Application filed October 16, 1915. Serial No. 56,184.

*To all whom it may concern:*

Be it known that I, ARTHUR E. SPINASSE, a citizen of the United States, residing at Mount Vernon, in the county of Knox and State of Ohio, have invented certain new and useful Improvements in Methods of and Apparatus for Drawing Glass; and I do hereby declare the following to be a full, clear, and exact description of the invention, such as will enable others skilled in the art to which it appertains to make and use the same.

The present invention relates to a novel method of and apparatus for drawing glass. It consists mainly in effecting the segregation of a portion of glass from a molten glass bath by means of a suitable element or drawing ring without, in general, permitting adhesion of the glass to said ring to occur.

My invention consists in chilling a part of the surface portion of a mass of molten glass, and drawing an article from or near the chilled portion; and in practice I segregate a part of said surface portion and either simultaneously with the act of segregation or later, chill the margin of said segregated portion and draw the article from within said margin. My invention also covers the apparatus.

Although within the broad scope of the invention other material may be used in making the segregating element, I choose to employ a metal, preferably iron, for this purpose. Also adhesion, in some degree may be permitted at times, and the temperature of the glass at the adhesive juncture regulated.

Heretofore refractory rings have been used, their upper edges, or rims, have been made to project above the surface of the glass. I have discovered that the portion of glass adjacent and in contact with the floating or projecting portion of the ring is liable to become impaired, and at times crystallized. It becomes rough and hard, and is very adherent to the ring and is liable to be drawn into the object causing breakage of the latter. A skimmer is sometimes used to remove this adherent glass but this produces a number of other blemishes and defects.

The adhesion to rings of the kind referred to is also very great, and the ring must be reheated to a high temperature, which occasions serious delay. It is necessary also

to use a large number of tools and expend much labor and time in effecting this reheating to melt out and clean this impaired adhering glass.

My segregating element is cold, or comparatively so, remains clean, and has many other advantages; in fact I regard it as marking a new step or departure in the art of drawing glass.

Many ways of drawing glass are possible. I may draw from a deep, semi-deep, or shallow body of glass. I may or I may not reheat the place or point from which I draw to reduce residue glass. I may also use in conjunction with my said segregating ring, a secondary ring of refractory material.

My invention contemplates various other features which may be detailed below.

In the accompanying drawings:

Figure 1 is a vertical view through the forehearth of a glass furnace, showing my segregating element in position.

Fig. 2 is a top or plan of the same or a similar forehearth.

Fig. 3 is a section on the same line as Fig. 1, showing the segregating element raised after the completion of a draw.

Fig. 4 is a similar section showing said element raised further and a cover in place.

Fig. 5 is a side view in section, showing one form of my complete apparatus, taken on line A—A of Fig. 6, showing the drawing chambers partly outside and partly within the body of the tank furnace. Fig. 6' is a section on the line D—D in Fig. 6.

Fig. 6' is a view of a detail.

Fig. 6 is a top view on line C—C in Fig. 5.

Fig. 7 is a sectional view on line B—B in Fig. 5 and Fig. 6.

Fig. 8 is a detail perspective view of one of the bricks which I may employ in my regenerative furnace.

Fig. 9 is a section on the line a—a in Fig. 8.

Figs. 10 to 13 are sectional views illustrating ways in which my segregating element may be employed.

Fig. 14 is a top or plan view of a modification of the upper part of the apparatus shown in Fig. 5.

Fig. 15 is a side view of the portion of the apparatus shown in Fig. 14; and

Figs. 16 to 27, inclusive, are sectional

views showing modifications in structure and use of my segregating element or cooled metal shield supporting member, the slabs supported by said element and the sub- 5 merged plate or refractory element.

The broad features of my device are shown in Figs. 1 to 4.

In Fig. 1, 1 is a glass melting tank of a common type with a forehearth or drawing 10 chamber 2. The top of said chamber, as in Fig. 5, may, with a portion of the tank wall, recede within the tank furnace body and form an alcove above the glass, it is suitably covered by a sectional roof or slab 3, where- 15 in is provided opening 7. Arch 8 above the level of the glass 9, provides for the free passage of hot glass and continuous heat from the main furnace. A forehearth 2, preferably of semi-shallow depth, is shown. 20 The body of the glass 14' in the forehearth or drawing chambers is with great ease maintained at high temperature, owing to the fact that it is in uninterrupted communication with the mass of molten glass 9, 25 within the main tank furnace 1. Because of this fact, any floating element or aftermath from a preceding operation may readily be moved or floated from the drawing kiln to within the tank furnace where it is rapidly 30 reheated and purified by subjection to the deep heated atmosphere and the large mass of molten glass therein.

The numeral 5 indicates a ring of metal, preferably iron or steel, with its lower end 35 10 smoothly polished and having a rounded tapering downward edge; it is hollow and fluid cooled, and is adapted, by means of suitable supports, such as its cooling fluid feeding pipes 11 and 12, to be moved into or 40 from the glass. Other supporting means may be used.

The ring may be lowered so that the lower portion 10 becomes immersed to a suitable depth in the body of molten glass 9. Cooling 45 fluid, such as water, is caused by means of feeding pipes 11 and 12 to circulate through it to maintain the same at a temperature low enough to avoid adhesion of the glass in contact therewith as indicated 50 at 13 in Fig. 1. The portion of glass in contact with the ring and that adjacent thereto, is cooled in proportion to the temperature and character of the cooling medium forced through the ring, thus forming 55 a non-adhesive shell of glass which I have indicated by numeral 14, in Fig. 3, and which segregates the portion or area 15 from which the glass article 16 is being drawn by means of a drawing or blowing 60 apparatus.

I am therefore able to draw glass rapidly and properly within this cooled shell of glass; and, what is of great importance, I may, without interfering with my drawing 65 temperature, maintain the outer area sur-

rounding the ring as at 14', at a high temperature..

In Fig. 2, a top plan view of Fig. 1, I show the preferred sectional protecting slab or roof 3. I may use burners 21 and 22, but 70 preferably I use burners 17 and 18, so that the end of the flame or heat generated may travel with the current of the glass and toward the front wall of the kiln.

In Fig. 3, a fractional view of Fig. 1, I 75 show the non-adhesive and vertically movable metallic glass segregating ring 5, elevated, the cylinder 16 separated from the glass bath by heat or otherwise, and, because of the shape of and smoothness of the 80 lower portion of the ring 5, and because of the temperature thereof and the fact that it is free from adhesion, no glass from the bath is lifted with the walls of the ring and the part 14 separated from said ring is not 85 considerable. This portion 14 remains floating on the surface, whence it may be removed together with residue glass toward the front or out of the tank or forehearth in the direction of the arrow, leaving a clean 90 surface for a succeeding operation of drawing. However, as shown in Fig. 4, I prefer to shove this portion 14 within the melting zone of the tank, as shown at 23, where it is 95 remelted. This removal is effected by means 95 of a skimming tool 24, by unskilled labor. Thus at once I obtain a clear space beneath the ring free from dripping glass from said ring which allows of the immediate skimming or melting of the refuse glass at the 100 surface and without delay I provide a clean surface at 25 to repeat the drawing operation.

If desired, however, the element 5 may be further elevated and a lid 26 placed over the 105 drawing opening 7, as shown in Fig. 4.

It is evident from the foregoing that the operation of drawing may be practically continuous, and generally the top of the deep or shallow body of glass, as may be the case, 110 need not be reheated between operations, but simply a portion of the top surface at least as large as the area affected by the segregating ring is cleared of impurities or incompletely melted glass by means of the 115 skimmer tool referred to.

Of course this invention may be used with any form of tank or forehearth containing glass.

In Figs. 5 to 9 I show further modifications of structure and modes of operation, the tank furnace 1, the space 28 under arch or base of wall 8 in the rear of the drawing kiln, which kiln or drawing chamber as clearly shown to a degree projects outwardly 120 from the main furnace wall and also, in suitable degree, recedes within the body of said tank furnace so that the glass body in the drawing chamber is maintained in high melted condition and pure. This is 125 130

also due because of the free space provided under the recessed arch or wall 8, and because of the fact that the forehearth is constructed with walls free of obstruction or projection on the interior, the surface of the glass 9 being as in Fig. 1 free from any obstruction, floating elements may be moved from one compartment to another and because of the fact that the space in the rear 5 of the kiln is at least as large as the front part therein, it will be noted that the cover or roof 3 with the opening 7 conforms in construction with the drawing chambers and also extends in somewhat outside the 10 tank furnace and transversely recedes within the tank furnace, opening therein preferably receding not beyond the breadth line of the furnace wall body.

31 is a floater or gate which may be used. 20 It is vertically operated and maintained in suitable position by rods 32 of fire resisting material. These rods are inserted in openings 33 provided at each end of the floater. I provide rods 35, provided with 25 sockets 34 and turn buckle 36 which engage the rods 32, and bent levers 39, 40 and connecting rods 41, 42 provided with counter-weight 43, serve to operate the floater. I provide this mechanism in any number, 30 preferably two in this case, for independent raising or depressing either end of the floater.

It is clear that by lowering or raising 35 any of the rods 42 the floater 31 may be lowered or raised accordingly to desired position, and may be submerged in the body of glass. This is advantageous in controlling the character of the glass as to fluidity as it passes to the drawing point, and in 40 freeing the surface of the glass from impurities. The floater may be held in any desired adjustment by means of a pin in any of the holes 43' in rod 42.

44 is a ring or an open bottomed pot 45 made of refractory material. I provide rods 46 of refractory material, and these are adapted to engage openings 46' in extensions 45 from the rim or edge of said pot so as to hold the ring or pot 44 submerged 50 in a suitable position, and at a suitable depth below the drawing opening. The ring or pot 44 may, of course, be provided with a greater number of extensions 45 than the two shown, and such additional 55 extensions made to project from said ring or pot at various points therearound in order to secure the desired vertical adjustment or cant; and with each such extension should coöperate an additional rod 46. 60 Rods 46 are held by rods and sockets 47, which in turn are held in position by means of bolts 48 in beams 48'. However, I may use in connection with each rod a mechanism such as that which operates the floater 31, in 65 order that the centrally opened bottom pot or

ring may be quickly brought to the desired plane position, vertically or maintained in position in relation to the surface of the mass of glass. In connection to this I prefer to use my device shown in Fig. 26, as a shield 70 lowered near the surface of the glass body as per description Fig. 21, or adjacent with the upper surface of the ring or pot.

In Fig. 6' I show my submerged pot 44 maintained with its flange 45 near the surface of the glass bath 9 by means of rods 46 engaging openings 46' in the flange 45. These rods may be two or more in number and are connected to independent mechanisms or means such as that which I use to 80 operate floater 33, as shown in Fig. 5. Therefore the pot may be raised or depressed at different points to cause it to assume positions suitable for drawing. As before described, 3 is the roof having a 85 drawing opening 7. A refractory shield, made up in sections 52, rests upon the hollow water-cooled metal support 5, which is provided with inlet and outlet pipes 11 and 12 connected to a water supply and to raising and lowering means. In this case, as in Fig. 21, I show the support 5 and shield lowered through opening 7 near the surface, but not in contact with the glass bath. This is sufficient to shut off excess furnace heat 90 from the drawing area, where I show the cylinder 16 in the process of being drawn by means of drawing tool 16'. After drawing, the shield and its water-cooled support beneath are raised preferably above the furnace to expose the drawing area to the furnace heat. The bath surface is then skimmed or cleaned from refuse glass and the drawing operation is repeated. This 95 cleaning, it will be seen, is rapid and efficient, due to the fact that the surface of the bath remains unobstructed by the projecting clay member which not only has a great tendency to destroy the quality of the glass, but further prevents the efficient and rapid 100 cleaning which, in my present method and apparatus I so readily obtained.

Around the walls, or preferably in the front part of the forehearth 2, I provide a regenerative system arranged to reheat the gas 115 and the air by which is burnt the gas, which I use as fuel. The products of combustion pass down through channels 49 to the flue 51. These channels, which are built with refractory brick are highly heated and thereby serve to preheat the air and gas, as shown in Fig. 7, entering through channels 56 and 57, arrows pointing the course of the agents of combustion which are burned in the space above the glass, and of the consumed gas to the flue 51, whence it goes to the stack.

Gas may be forced through channel 56 and air through channel 57, and both may be mixed at any point desired. Both of 120 125 130

these channels may be used for the air, however, and gas introduced at 54. I do not here claim a regenerative system, but I do here claim its adoption in connection with 5 a forehearth or tank for drawing glass; and the advantage of this will be apparent to any one skilled in this art. It is also of special value where artificial gas is used, as it could not very well be used with a common 10 burner. The use of a regenerative system with a drawing forehearth is of great value, as it enables me to get a purer and hotter fire.

Referring again to Fig. 5, the ring 5 is 15 shown supporting a grooved ring 52 of refractory material, which, as shown in Fig. 6, may be made in sections. This ring 52 is to prevent cooling by radiation aside from the point of contact of ring 5 with the glass. 20 Ring 5, as stated, is supported by suitable means, in this case its own pipes 12 and 11, and these are suspended by means of cables 59 and 60, for free vertical movement by means of drum 61 and motor 62, which motor should be capable of being reversed so as to give motion to the cables in both directions. The ring 5, therefore, supports the grooved ring 52, thus eliminating much breakage. As shown in Fig. 6 there are six 25 sections of this ring 52, but it may be integral as well, and should be supported in easy relation to the segregating ring 5.

The submerged ring 44 below may form 30 an anchorage for the glass flowing therein through opening 53. After drawing ring 5 is elevated, as explained, the cylinder separated, the floater 31 then submerged and the refuse glass floated within the tank for remelting, the floater may again be elevated 40 and ring 5 lowered for a succeeding operation. However, door 58 may be opened for cleaning and, with the aid of skimming tools, the refuse glass is pulled over spout 72 between the regenerators and falls into 45 a cellar through the well or pit 71, where it may be removed from time to time.

In Figs. 10 to 13 I have illustrated several 50 ways of drawing glass articles by means of my invention, though in these figures I show the drawing of a glass cylinder, within the broad scope of my invention a glass sheet or other glass articles may be drawn by similar means modified in form to correspond to the object to be drawn.

In Fig. 10, 3 is the top stone, 5 the ring 55 segregating a portion of glass and cooled by means of fluid circulated through said rings by means of pipes 11 and 12. As stated, 17 is a heat generating means. The arrows indicate the escape of a portion of the heat 60 outside of the ring around the cylinder to remove any stress imparted by the positive cooling of the cylinder at its base.

In my apparatus the drawing area is posi-

tively cooled by the segregating means, and 65 the cooling effect of this means is regulated at will; and further, the cooling effect of the segregating means by radiation, may be controlled at certain points and even practically prevented by the use of refractory 70 block 52 upon the said segregating means as shown in Fig. 5.

Now, the element 5 may be cooled to different degrees. It will be clear also that it is possible to cool the same more at one place 75 than another, if desired, and the interior of the ring may be divided into chambers for that purpose; and in fact while I here show the ring integral, it may be in sections, each section or chamber having its set of pipes 80 whereby one section or chamber may be controlled independently with respect to each other section or chamber. This is indicated in Fig. 26.

In the structure shown in Fig. 10, the 85 temperature of the ring is lowered so as to cool a portion of the glass, as indicated by the shade line 74, from which a cylinder 16 is being drawn.

In the showing of Fig. 11, the glass at 90 point 75 has been cooled to a greater extent as compared with Fig. 10, and the cylinder is being drawn with its base close to said point 75. To obtain this effect the ring is chilled faster, but the cylinder 16 is drawn 95 faster.

In the showing of Fig. 12, the temperature of the ring is so regulated in relation to the speed of the draw as to permit drawing the article directly from the ring at 100 point 76. That portion of the glass which is gradually cooled and formed by the ring is therefore drawn into the cylinder. The ring, therefore, is somewhat of an outer former, and should accordingly have a 105 smooth and polished surface. However, I may impart or stamp or print a design to the glass as drawn; for instance, by using a ring with vertical grooves 90, Fig. 27, I may produce ribbed glass.

In carrying out the method indicated in Fig. 13, I first bring the segregating ring to a suitable position in the bath, where it is allowed to remain for a time sufficient to form a cooled non-adherent shell of glass 115 thereabout, after which I start to draw the object 16 and at the same time lower the ring 5 which carries down therewith the cooled shell of glass as appears at 77. Thus, as shown, the cylinder 16 is drawn from the 120 glass which is fed upwardly, supplied by hydrostatic pressure, and inside this non-adhesive chilled shell of glass. Flat sheets of glass or other glass articles may be drawn in this manner by providing an oblong or 125 square drawing ring. I may bring my ring to a temperature to permit glass to adhere to the same when first lowered to position

77 and then suitably lower the temperature thereof so as to chill and fix the inner adherent glass in the form of a cooled layer to the ring, and then further lower the ring 5 and draw a glass article upwardly from the glass within said cooled adherent layer on the interior of the ring. Should a refractory ring be used, air should be used as a cooling medium. This way of using the 10 glass segregating ring is quite desirable for the drawing of sheets or plate of glass. I believe also that I am the first to provide a hollow circular water cooled element of oblong or rectangular form and contour 15 provided for cooling and also for raising or lowering the same, and I hereto claim the use of said device in its broad scope of application in glass drawing.

Other modifications of the process and 20 apparatus may be employed, and glass as heavy as plate glass may be rapidly drawn and be free from the blemishes often produced during the old process of drawing. The problem of removing these blemishes has 25 been a vexatious problem of long standing.

Within the broad scope of my invention the cooling fluid in the ring may be decreased to a point as to permit adhesion, and the temperature and nature of the adhesion 30 regulated. The ring may be cleaned and greased before each operation when the glass is not permitted to adhere.

In case the glass is permitted to adhere, the glass is simply melted away from the 35 ring after the draw is completed. The ring, however, during drawing is kept at a temperature sufficient to prevent any of the metal melting off or mixing with the glass in the forehearth.

40 In the structure of Figs. 14 and 15, 48' are the supporting beams, 61 the winding drums, and 62 the motor, as already referred to. I provide a U-shaped frame 83, which frame carries the pulleys over which the 45 cables pass to the winding drums, and which, by means of wheels 84 and 85 provided with screws taking into brackets 86, may be moved laterally so as to adjust the position of the ring 5 in relation to the drawing tool 50 16' as indicated in Fig. 6. It may be operated from below by connections similar to the one used to operate the floater in Fig. 5.

The above described features which provide for the lateral adjustment of the supporting means for the shield or cooling member 55 and the vertical adjustment of said shield or cooling member from and to a point above the surface of the molten glass are shown, described and claimed in my co-pending application, filed February 11, 1920, 60 Serial Number 357,984.

In Fig. 16 I show a segregating ring enlarged in vertical dimension at 77' adapted to penetrate deeper into the glass on one

side and gradually less on the opposite side 65 where it may even rise to a position level with or slightly above the surface of the glass, according to the lowered position of said device. Outside this is shown submerged a ring 78, with the rods 46 directly 70 engaging the top thereof at desired points.

In Fig. 17 I show a segregating ring enlarged horizontally at 79. Inside is seen a submerged ring 80.

In Fig. 18 I show the ring provided with 75 a flange 81 for preventing dirt falling into the molten glass. 82 designates a narrow slab under one side of the said ring.

In Fig. 19, as in Fig. 16, I show a ring enlarged in vertical dimension at one place, 80 but in place of projecting into the glass the larger portion 83' of the ring in this case projects upwardly. Ring 84' is made to penetrate more deeply on one side than on the other. 85

In Fig. 20 I show the segregating element having a flat bottom at 85' and lowered merely to come into contact with the surface of the molten glass at 86'. Underneath may be a ring 87, heavier or thicker 90 on one side as at 88.

In Fig. 21 I show a member similar to that of Fig. 20, lowered near the surface of the glass 86', but not in contact therewith. It is brought to just the point where it prevents excess transfer of heat by absorption of the ring, this member may as in Figs. 5, 22, to 25, support a refractory ring or shield device. A ring 87 may be used in this instance. 95

The lop-sided feature common to many of the various forms just discussed is designed to afford an opportunity for effecting compensation for uneven temperatures in the glass, so as to procure at the drawing 100 zone uniformity of temperature and hence homogeneity and uniformity of viscosity.

The ring at 77', extending deeper on one side than the other, cools the glass in the drawing process, on the deep side, further 110 down, at the same time permitting on the furnace side, glass from a slightly greater depth to enter the ring, this glass from the greater depth approximating the temperature and viscosity of the glass from a shallow stratum on the other side. The ring 83' also has a similar effect, when taken in connection with the refractory ring 84', which ring projects deeper on one side, and which, as pointed out above, may be substituted for pot or ring 44, and which, as indicated, may, by means of mechanism similar to that which actuates floater 31, be, like said floater, adjusted to any desired position in or above the glass. The deeper 115 vertical part to the right or tank side, helps to insure the inflow of slightly cooler and thicker lower layers of glass, as well as pro-

viding a shield slightly more effective on the tank side, than on the other.

The rings 5 and other refractory rings are, as indicated, interchangeable in their 5 relations throughout.

The outer horizontal top flange shown in connection with ring 84', assists in keeping the ring floating level, and practically counteracts the cant which the ring would otherwise have a tendency to assume, if floating with the flanges partly above the surface of the glass, owing to the greater buoyancy of the deeper side. The flange thus keeps the upper edge of the ring practically parallel with the surface of the glass. This flange also, when floating partly above the glass, affords means for holding the ring in proper position, and also protects the glass surface outside the drawing zone, from falling impurities.

In Fig. 22 I show the top of the metal ring supporting a refractory heat retaining ring shield of suitable height.

These features described above relating to 25 the uneven shaping or dimensions in vertical cross sectional area of the shield, cooling member or segregating member are shown, described and claimed in my application filed February 11, 1920, Serial Number 30 357983.

In Fig. 23 I show the top and one side protected.

In Fig. 24 I show the top and both sides protected by a refractory top which extends 35 some distance outward.

In Fig. 25 I show the outside and the top of the ring protected by a refractory slab extending outwardly.

In Fig. 26 I show a half portion of a 40 circularly arranged device composed of independent hollow curved metal sections or members 5 or 5'. I provide these hollow members in any number, preferably 3 to 4, and they may be of any desired form or 45 contour so that when assembled, as shown they form a device of circular, oblong or other desired contour and corresponding to the opening 7, or to the form of the article to be drawn. Each of the independent hollow metal members is provided with independent fluid cooling means, preferably inlet and outlet water cooling pipes such as pipes 11 described in Fig. 5; thus the members are cooled independently. The members are also conjointly or independently provided with raising and lowering means such as parts 59, 36, 61, 62 together with other means shown and described in Fig. 5, each hollow metal water cooled member is 50 therefore independently adjustable and because of this, and of the fact that they are independently cooled as the case may require, a great number of important advantages are obtained which could not be seen 60 cured with a ring of integral form, due to

the fact, as stated, that, the sections forming the ring or device may be caused to assume different relative positions to meet the changing conditions always in the process of drawing glass mechanically. This 70 device can, with great advantage, be used as a shield but with advantage as a shield supporter and each member may be provided with a corresponding section of heat retaining refractory shield of fitting form 75 and suitably supported by said member in a way shown in Figs. 5, 22, to 25, of course other arrangements are possible.

In Fig. 27 I show a ring with vertical corrugations 90, for the production of ribbed 80 glass.

The foregoing shows the various ways in which my cool drawing ring or segregating element may be modified. Thus I am enabled to cool one part more than others by 85 making my ring in sections and by introducing more of the cooling agent into one section than into others; or I may make my ring so as to hold more of the cooling agent in one portion of a single channel, as in 90 Figs. 16, 17, 19, than in others, and I may modify the shape of the supported slab to the same end. I may further cool or modify the character of the glass at different portions of the generating cylinder to obtain 95 uniformity of walls. I may produce like effects by changing the shape and position of the submerged plate.

I desire my invention to cover all modifications within the scope of the same, whether 100 said modifications have been described or not.

What I claim as new and desire to secure by Letters Patent is:

1. In glass drawing apparatus, a hollow metal segregating device having sloping polished walls, and means for circulating cooling water through said hollow metal segregating device to maintain the same at a temperature low enough to avoid adhesion 110 of the glass in contact therewith.

2. In combination with glass drawing apparatus, means adapted to take position in a glass bath and surround a portion of said bath, said means adapted not to adhere to 115 the glass and constructed with walls of such contour and surface that the same may be withdrawn from the bath after drawing without retention of glass, and a device for raising and lowering said means to and from 120 the glass bath.

3. In combination, a hollow metal member adapted to take position in a glass bath and surround a portion of said bath, said member constructed with walls of such contour 125 and surface that the same may be withdrawn from the bath after drawing without retention of glass, means for circulating water through said hollow metal member to maintain the same at a temperature to pre- 130

vent adherence to the glass, and means for lowering and raising said member to and from the glass bath.

4. A hollow metal segregating device having polished walls shaped to shed the glass as it is in the act of being withdrawn from a glass bath, means for circulating cooling water through said hollow segregating device at a temperature low enough to prevent adherence of the glass to said polished glass-shedding walls, and mechanism supporting said device for raising and lowering the same to or from the glass bath.

5. In glass drawing apparatus, the combination of a drawing chamber containing molten glass and having a space above the glass for the circulation of heat, a metal ring adapted to segregate a portion of the molten glass without adherence thereto and projecting up through said space to protect the drawn object from the circulating heat.

6. In glass drawing apparatus, a hollow metal segregating device, means for circulating cooling water through said device whereby to maintain said device at a temperature to prevent its adherence to molten glass, a refractory shield supported upon said device, and means for supporting and for raising and lowering said member and shield with respect to a glass bath.

7. In glass drawing apparatus, a glass-segregating member comprising a hollow metal annular member adapted to be withdrawn from a glass bath between drawing, the walls of said member being constructed with a contour and surface so as to avoid retention of glass when it is withdrawn from the bath, means for circulating cooling water through said member to maintain the same at a temperature to prevent said walls from adhering to the glass of the bath, and means supporting said member for raising and lowering said member to and from the glass bath.

8. In glass drawing apparatus, the combination of a tank furnace containing a molten glass bath and having a drawing opening spaced above the glass, a hollow metal glass-segregating annular member having smooth walls to prevent marring the glass and also to assist in preventing said walls from adhering to the glass of the bath, means for circulating cooling water through said member to maintain the walls of the same at a temperature low enough to insure avoidance of adhesion between said walls and the glass of the bath, the walls of the member being constructed to taper downwardly so that they will not retain any glass when the member is withdrawn from the bath after drawing, means supporting the member for raising and lowering said member through said opening into and from the glass bath, and means for drawing a glass

object from the glass within said member when lowered into segregating position and upwardly through said member, the object being shielded from the furnace heat by said member which extends upwardly to said drawing opening of the tank furnace.

9. In an apparatus for drawing glass articles, a drawing tank furnace containing a bath of molten glass, said tank having a drawing opening, a hollow metal member adapted to be immersed in the bath and to surround a top portion thereof, means for circulating water through the walls of said member to maintain said walls cooled below the point at which they will adhere to molten glass, a refractory shield supported upon said member and extending upwardly to the drawing opening when the member is lowered to segregating position, means for drawing a glass object from the segregated portion of glass, the glass object being protected from both the cooling influence of said member and from the furnace heat by said refractory shield, and means supporting said member for raising and lowering said member together with the shield through said opening to and from the molten glass bath.

10. In a glass drawing apparatus, in combination, a chilling segregating device, a grooved heat retaining device fitted over said segregating device, and pipes for circulating a chilling means attached to said segregating device and supporting it.

11. In glass drawing apparatus, a refractory shield, and water-cooled glass segregating ring means directly supporting said shield.

12. In glass drawing apparatus, a refractory shield, and cooled glass segregating ring means receiving the weight of said shield and supporting said shield from beneath.

13. In glass drawing apparatus, a hollow metal glass segregating member, means for circulating cooling fluid through said member, and a shield supported on said member and adapted to protect the drawn object from the cooling action of said hollow member.

14. In glass drawing apparatus, a refractory ring shield a hollow metal glass segregating ring supporting said shield and adapted to receive a circulation of cooling water therethrough and means directly attached to said metal ring for raising and lowering said ring and supported shield.

15. In glass drawing apparatus a refractory ring shield a hollow metal glass segregating ring placed beneath and forming a continuous support for said shield to prevent sagging, said hollow metal ring adapted to receive cooling water whereby to protect itself and the shield from injury caused by excessive heat, and means attached

- to said metal ring for supporting said shield without direct connection therewith, said means also adapted for raising and lowering said shield.
- 5 16. In glass drawing apparatus, an annular shield made up in sections, a hollow metal member adapted to support the shield sections in an upright position from beneath, means for circulating cooling fluid through 10 said metal support, and means for lowering said support together with said shield sections thereon.
17. In glass drawing apparatus, a drawing tool, a drawing chamber in free communication with a tank furnace and adapted to be supplied with glass from said furnace, said chamber having a drawing opening for drawing a glass cylinder spaced above the glass, a ring shield member of a dimension less than said drawing opening, and 20 cooled means for supporting the shield and for raising and lowering said shield through said opening with respect to the glass in said chamber.
- 25 18. In a glass drawing apparatus, a refractory body adapted to be submerged beneath the surface of the glass, and means whereby it may be shifted in the bath of glass to vary its depth beneath the surface 30 of the glass so as to control the fluidity of the glass for the drawing operation.
19. In glass drawing apparatus, a refractory body adapted to be submerged beneath the drawing surface in a glass bath, 35 said refractory body being flat and having a centrally depressed portion formed with a spherical wall, said refractory body also having a central opening at the base of the spherical wall to admit glass, extensions on 40 said refractory body, and means for engaging said extensions to maintain the refractory body submerged beneath the drawing area and to change the vertical position of parts of said refractory body with respect to 45 other parts thereof.
20. In glass drawing apparatus, the combination of a tank furnace containing molten glass, a forehearth having an opening connecting same with said furnace, a refractory body immersed in the glass in the opening 50 between said furnace and forehearth, and means for depressing said refractory body below the surface of the glass and keeping it there.
- 55 21. In glass drawing apparatus, a tank furnace containing molten glass, a drawing chamber communicating with the furnace, a floater between said furnace and drawing chamber, and means for adjusting the vertical 60 position of said floater in the glass to regulate the temperature of the glass as it passes from the furnace to the drawing chamber.
22. In drawing apparatus, a hollow metal 65 segregating device, means for circulating cooling water through said hollow segregating device to maintain the same at a temperature that will prevent its adherence to glass, a refractory body adapted to be submerged in the glass bath beneath the drawing area, said refractory body having an opening therein through which the glass may pass, and means for shifting said refractory body in the bath to change its position with respect to the drawing point, so as to control the character of the glass as to fluidity.
23. In glass drawing apparatus, a glass segregating means adapted not to adhere to the glass, a refractory body adapted to be submerged beneath the surface of a glass bath and adapted to be shifted in the bath to vary its position with respect to the drawing point, so as to control the character of the glass as to fluidity, and means for lowering 85 said segregating means to segregating position in the bath and for withdrawing said segregating means out of the glass bath.
24. In a glass drawing apparatus, in combination, a chilling segregating device 90 adapted to be partly immersed in the molten glass, and an open bottomed pot adapted to be held immersed below the said segregating device.
25. In a glass drawing apparatus, in combination, a hollow chilling ring, means for causing circulation of a chilling medium through said ring, means for holding it partly immersed, an open bottomed pot, and means for holding said pot submerged below 100 said chilling ring.
26. In glass drawing apparatus, the combination of a glass tank furnace, a drawing chamber communicating with said furnace, glass segregating means adapted not to adhere to the glass and arranged to be immersed in the glass in said drawing chamber, a refractory body immersed in the glass between said drawing chamber and furnace, and means for adjusting said refractory 110 body vertically in the glass.
27. In a glass drawing apparatus, in combination, a chilling ring, means for drawing glass from within said ring, a forehearth into which the said ring may be lowered, a floater arranged between the forehearth and the furnace, means whereby the floater may be depressed below the surface of the molten glass, and an opening in said forehearth wherethrough the detached end of a draw 120 may be shoved from the forehearth over the floater into the main tank.
28. In glass drawing apparatus, the combination of a furnace, a drawing chamber communicating with said furnace, a refractory body adapted to be submerged in the glass in said drawing chamber, said refractory body having an opening through which the glass may pass, means for shifting the 125 position of said refractory body and for 130

- holding it in shifted position, a floater disposed between said furnace and drawing chamber, and means for moving said floater vertically in the glass.
- 5 29. In glass drawing apparatus, a glass tank furnace, a drawing chamber communicating with said furnace, a hollow metal segregating device, means for circulating water through said device to render same non-adherent to glass, means for lowering said device into the glass bath in said drawing chamber and for withdrawing said device from the chamber, a refractory body adapted to be submerged in the glass bath in said chamber and having an opening through which the glass may pass, a floater disposed between said furnace and drawing chamber, and means for shifting said floater vertically in the glass and for holding it.
- 10 30. An apparatus for drawing glass cylinders from a mass of molten glass comprising a tank for containing the molten glass and having an opening spaced above the molten glass through which the glass cylinder may be drawn, a refractory segregating member in the tank beneath the drawing opening, a ring shield, means for supporting said ring shield whereby it may be lowered through said opening to a position for drawing and whereby said shield may be raised between drawing operations, and independent adjustable means for holding the refractory member in predetermined positions for controlling the fluidity of the glass, said refractory member being free from connection or contact with said shield when said shield is in position for drawing.
- 15 31. In glass drawing apparatus, a glass tank furnace, a drawing chamber in free communication with said tank, a fixed roof to said chamber having an opening spaced above the glass in said chamber, a refractory ring shield, a hollow metal member supporting said ring shield from beneath, means for circulating cooling water through said metal member, means for supporting and for raising and lowering said member together with said refractory ring shield supported thereon through the roof opening of said chamber, a refractory pot or ring submerged in the glass in the chamber, means for causing vertical movement of said pot or ring and also for holding said pot or ring in desired submerged position relative to the surface of the glass, means for drawing a glass article from the glass above said submerged pot or ring and upwardly through said member and ring shield when the latter are lowered into position for drawings.
- 20 32. In combination with glass drawing apparatus, a refractory ring shield having a groove in its bottom, a hollow metal water cooled support fitting said groove and extending beneath said ring shield, means for circulating cooling fluid through said sup-
- port, and means for raising and lowering said support together with said ring shield thereon.
33. In glass drawing apparatus in combination a hollow metal water cooled ring, a refractory ring shield adapted to lie supported upon and on the sides of said metal ring, and means for circulating water through said hollow metal ring, said water circulating means adapted to raise and lower said metal ring with said shield thereon.
- 70 34. In glass drawing apparatus in combination a hollow metal water cooled glass-segregating device, a refractory shield supported by said device and means for circulating a cooling fluid into and through said segregating device, said circulating means being adapted to raise and lower said device.
- 80 35. The method of drawing glass articles which consists in circumscribing a definite area of the upper part of molten glass with a cooling agent, applied so as to absorb heat from the border of the area so circumscribed whereby the glass in said border and that enclosed thereby is made to become viscous, effecting substantial equality of viscosity within said circumscribed area by withdrawing more or less heat from the viscosity of any portion less or more viscous than is desired by varying locally the effect of the cooling agent and drawing articles from the area so circumscribed.
- 85 36. The method of drawing glass articles which consists in segregating a portion of molten glass without adhesion thereof to the segregating means, chilling the boundary portion of said segregated portion, drawing an article from said segregated portion, removing said segregating means from the glass, freeing the body of glass from chilled glass, and repeating.
- 90 37. The method of drawing glass articles which consists in segregating a portion of molten glass without adhesion thereof to the segregating means, chilling the boundary portion of said segregated portion, drawing an article from said segregated portion, removing said segregating means from the glass, reheating the surface of said glass, freeing said reheated surface portion from the remnants of the previously drawn article, and repeating the operation.
- 100 38. In the manufacture of glass, the steps which consist in segregating a portion within the upper part of a mass of molten glass with a segregating means, and imposing on said means a condition which will prevent adhesion between the glass and the walls of the segregating means that come in contact with such glass.
- 110 39. The process of drawing glass objects consisting in producing a portion of relatively low temperature, in a glass bath by surrounding a portion of the bath with a hollow metal member in contact therewith,
- 115 120 125
- 130

circulating cooling fluid through the member so as to obtain a temperature of the member low enough to prevent its adherence to the glass and to cool the glass in contact therewith, and drawing an object from the surrounded portion of glass within said member.

40. The method of drawing glass articles from a bath of molten glass with a segregating device, which consists in conditioning the walls of the segregating device which come in contact with the molten glass to prevent adherence between such walls and the contacting molten glass, cooling the margin 5 of the portion of the glass bath segregated by the device, and drawing an article from within the cooled margin.

41. The method of drawing glass articles by means of a glass segregating device which 20 consists in maintaining said device at a temperature to avoid adhesion of the glass, lowering said device to a predetermined position to segregate a part of the surface portion of molten glass, retaining said segregating device at such position for a predetermined time necessary to cool the margin of said segregated surface portion, thereafter further lowering said device to bring the inner cooled margin of glass below the level of the 25 mass of glass outside the device, and drawing an article from the glass supplied by hydrostatic pressure within said cooled margin of glass.

42. The method of drawing glass with a 30 hollow metal segregating device, which consists in circulating cooling water through said hollow metal segregating device to maintain the same at a temperature low enough to avoid adhesion of the glass in 35 contact therewith, segregating a portion of a mass of molten glass by immersing said device, and drawing an object from the segregated portion.

43. The method of drawing glass which 40 consists in polishing the glass-engaging walls of a hollow metal segregating device, circulating cooling water through the walls of said hollow segregating device at a temperature low enough to cool the segregating 45 device whereby to prevent its polished walls from adhering to molten glass, segregating a portion of a mass of molten glass by immersing said device, and drawing an object from the portion of the glass within said 50 segregating device.

44. In the manufacture of glass objects, the steps which consist in segregating a top portion of a molten glass bath with a segregating member to which the glass of the 55 bath will not adhere, drawing to form an object from the segregated portion of glass, withdrawing the member from the bath after drawing without lifting therewith any glass from the bath, restoring the surface of

the bath to drawing conditions, and repeating.

45. In the manufacture of glass objects, the steps which consist in surrounding a top portion of a molten glass bath in a tank furnace with a segregating member to which the glass of the bath will not adhere, drawing to form an object from the so segregated portion of glass, withdrawing the member from the glass and furnace after drawing without lifting therewith any glass from the bath, reheating the drawing area to restore the glass to drawing condition, and repeating the operation.

46. In the manufacture of glass objects, the steps which consist in surrounding a top portion of a molten glass bath with a metal ring at a temperature sufficiently low to prevent its adherence to the glass of the bath which comes in contact therewith, cooling the boundary portion of the segregated portion of glass, drawing to form an object from the so segregated portion of glass, withdrawing the member from the bath after drawing without lifting therewith any glass from the bath, floating the residual cool glass resulting from the operation to a melting point away from the drawing area to restore said area to a drawing condition, and repeating the operation.

47. The method of drawing glass articles with a hollow metal glass segregating device having its depending walls constructed to avoid supporting any glass, circulating cooling fluid through said device to maintain the same at a temperature low enough to prevent its adherence to hot glass, immersing the device at such temperature to segregate a portion of a glass bath, causing the glass of the bath in contact with the surface of the device to form a cooled shell of glass non-adherent therewith, drawing a glass object from the segregated glass within said shell, withdrawing the device from the bath after drawing without lifting the cooled shell from the bath, removing the shell together with the residual glass from the draw away from the drawing area to restore said area to drawing conditions, and repeating the operation.

48. The herein described method of drawing glass objects from a bath of molten glass in a tank furnace with a metal segregating device, which consists in maintaining the device during the operation at a temperature sufficiently low to cool the glass and prevent its adherence to the glass, immersing the device while being at such temperature in the bath to segregate for drawing a constantly replenished portion thereof surrounded by said device whereby the glass is cooled to drawing temperature but non-adherent to said segregating device, maintaining the glass within the furnace at high tem-

perature, and drawing an object from said segregated portion of glass while protecting the object drawn from the high temperature within the furnace during drawing.

- 5 49. The method of drawing glass objects with a hollow metal smooth-walled glass segregating and forming device, which consists in circulating a cooling agent through the device to lower the temperature of said 10 device sufficiently to prevent its smooth walls from adhering to molten glass, segregating and forming a relatively cool portion of glass from a mass of molten glass by means of said device, and drawing a glass object 15 from said portion of glass as it is being fed by hydrostatic pressure from the mass of glass within the surrounding smooth metal walls of said segregating or forming device.
50. The method of drawing glass articles 20 from a glass bath contained in a tank furnace, which consists in conditioning a segregating device to prevent adhesion between said device and the glass of the bath, segregating with said device so conditioned a portion 25 of the glass bath without adhesion of the glass to the device, drawing an article from said segregated portion, shielding the drawn article from the direct furnace heat, withdrawing the segregating device from the glass bath after drawing without lifting 30 from the bath any of the glass therewith, restoring the bath to a condition suitable for drawing, and repeating.

51. The method of drawing glass objects 35 from a bath of molten glass which consists in maintaining a glass segregating element at a temperature to prevent adhesion of hot glass thereto, immersing said element under such temperature so as to segregate a non-adherent portion of glass from the bath and then drawing the object from the glass so segregated.

52. The process of drawing glass articles which consists in so conditioning a glass 45 segregating element that it will not adhere to hot glass, immersing said element while maintained in such condition into a bath of molten glass to segregate a portion of glass non-adherent to the said element during the 50 segregating act, and drawing the glass article from the so segregated portion of glass.

53. In glass drawing apparatus, a hollow metal member, having a series of chambers 55 adapted to surround a drawn glass object, each chamber of the series having inlet and outlet pipes for independent circulation of cooling fluid through the chambers for the purpose of cooling or modifying the character of the forming walls of the drawn 60 glass object at any desired points.

54. A method of drawing glass articles which consists in lowering a shielding device into drawing position, maintaining a

refractory segregating float submerged in 65 the molten glass and free from contact with said shielding device, drawing the article upwardly from the segregated glass through the shielding device, raising the 70 shielding device, cleaning the surface of the glass and repeating.

55. The method of drawing glass articles from a large bath of molten glass contained in a tank furnace, which consists in producing a shallow pool of relatively low temperature in said bath without separating 75 said pool from the surrounding body of the bath while maintaining said pool in communication with the mass of glass beneath, by submerging in said bath a bottom-aper-tured pot beneath the surface of the drawing area, exposing said area to the atmosphere, shielding said area from the furnace heat, drawing and then reheating the drawing area by exposure to the melting heat 80 of the furnace and freeing the surface thereof from residue glass to restore said area to drawing condition for a succeeding drawing.

56. The process of drawing glass objects, 90 which consists in lowering a shield through a drawing opening into a drawing chamber in position to protect the drawn object from the furnace heat, drawing an object from the glass bath, withdrawing the shield 95 from the chamber after the drawing operation, placing a cover over the drawing opening after the shield has been withdrawn to confine the furnace heat and exclude cooling air whereby to reheat and restore the 100 glass bath to drawing condition, and maintaining said shield exposed to the atmosphere outside of the chamber to cool the same during the reheating of the glass within said chamber.

57. The process of drawing glass cylinders which consists in lowering a hollow fluid cooled member through the drawing opening into the drawing chamber and into position adjacent the base of the cylinder 110 to be drawn, drawing the cylinder from the glass bath, withdrawing said cooling member from the drawing chamber after the drawing operation and while said cooling member is exposed to the atmosphere outside the chamber, placing a cover over the drawing opening to confine the furnace heat and exclude cooling air, whereby to reheat and restore the glass bath to drawing condition, then removing said lid and lowering 115 said cooling member for the next drawing operation.

58. The method of drawing glass articles which consists in segregating a portion of glass from the top part of a bath of molten 120 glass by means of a segregating element, the temperature of said element being reduced to affect the viscosity of the glass in

suitable degree or place peripherally, and drawing an article of glass from the so segregated glass within said element.

59. The method of drawing glass objects  
5 which consists in immersing a glass segregating element into a bath of molten glass to segregate a portion of glass from the top part thereof, regulating the temperature of said element in any degree or place to affect  
10 the viscosity of the segregated portion of glass, and drawing from the so regulated segregated portion of glass.

60. The method of drawing glass objects

which consists in immersing a hollow refractory glass segregating element into a 15 bath of molten glass to segregate a portion of glass from the top part thereof, applying cooling fluid in suitable degree and at suitable places to said element to affect the viscosity of the segregated portion of glass 20 at such places and drawing so as to obtain a glass object of desired form from the so segregated portion of glass.

In testimony whereof, I affix my signature.

ARTHUR E. SPINASSE.